

Jan. 1, 1929.

1,697,702

E. B. WESTON ET AL

PROCESS FOR MAKING WATERPROOF STRAW PULP BOARD

Filed Nov. 4, 1926



INVENTORS  
and EDWARD B. WESTON  
WILLIAM G. CLARK  
BY  
*J. Granville Meyer*  
ATTORNEY

## UNITED STATES PATENT OFFICE.

EDWARD B. WESTON, OF DAYTON, OHIO, AND WILLIAM G. CLARK, OF TERRE HAUTE, INDIANA, ASSIGNORS TO THE TERRE HAUTE PAPER COMPANY, OF TERRE HAUTE, INDIANA, A CORPORATION OF OHIO.

## PROCESS FOR MAKING WATERPROOF STRAW PULPBOARD.

Application filed November 4, 1926. Serial No. 146,153.

This invention is an improvement in straw board, and processes of making the same, and more particularly in moisture resistant straw board, especially adapted for use in 5 the manufacture of fibre packing and shipping containers, and wherein the strawboard sheets are corrugated and usually combined with attached facing and backing sheets.

Straw board is usually made by steam 10 cooking straw with a suitable alkali, such as lime, in a digester. The straw pulp as usually manufactured has an inherent tendency to foam in the paper making machine, and this tendency we have discovered is 15 very greatly increased by the addition of sizing, such for instance as rosin or colophony.

Heretofore, it has been impracticable, if 20 not impossible, to make moisture resistant straw board, because, as we finally discovered, of the reaction between the alkali remaining in the pulp after the usual washing and the sizing used in the water proofing process. The pulp tends to foam and become slimy, so that it will not cling or stick 25 to the cylinder of the paper machine.

We have discovered that by cooking in a 30 properly conducted manner and by eliminating all or substantially all of the alkali by careful and extended washing, this tendency 35 of the pulp to foam and to become slimy may be very greatly lessened, and that by reducing the agitation of the flowing pulp to a minimum, an excellent quality of moisture resistant straw board may be made on the usual paper making machine. That is by cooking in the manner to be later described, afterwards washing thoroughly, and making the flow of the pulp to the cylinder even 40 and uniform, the foaming may be eliminated, so that the pulp does not become slimy, and readily adheres to the cylinder.

One of the primary objects of the present 45 invention is the provision of a process for producing a water resistant straw board, wherein the water resistant substance is intimately incorporated with the material of the board while in the state of pulp, so that the board is throughout uniformly moisture 50 resistant, at the same time sufficiently flex-

ible or pliable to withstand the action of the usual corrugating rolls when the sheets are to be corrugated.

Another object is the provision as an article of manufacture, of a water resistant straw 55 board.

With these and other objects in view, the invention consists in the article and process of making the same, it being understood that the ingredients and nature thereof, as well 60 as the proportions may be varied within the scope of the claims appended hereto.

In the drawings forming a part hereof, is shown a diagrammatical sectional view of 65 a part of a paper making machine of the cylinder type, adapted for the making of the improved board.

In the usual process of making ordinary straw board, the straw is cooked in digesters 70 with an alkali, such as lime, by means of steam. In the present process the same procedure is followed, except that the cooking operation extends over a definite time, with a definite steam pressure, and with a definite quantity of lime. The cooking, which requires about 145 lbs. of lime to a ton of straw, is continued about ten hours, under about 30 lbs. steam pressure, and the operation is very carefully watched to attain precisely the quality of pulp desired. 75

After cooking, the pulp is subjected to an extended washing operation with clear water, until all or substantially all of the lime is removed. The washing operation is continued until little or no reaction is obtained 85 with the phenolphthalein test. When this result is obtained, the sizing is added to the pulp, and thoroughly incorporated therewith.

A preferred sizing material is rosin or 90 colophony and alum. In incorporating the sizing material with the pulp, the rosin is first added to the washed pulp in the beater and thoroughly mixed by the operation of the beater. The mordant, in the present instance alum, is then added, and the operation of the beater is continued until a complete mixture is obtained. The proportions of rosin and alum will depend somewhat on 95 conditions, such as for instance the charac- 100

ter of the water. A suitable proportion is about 90 lbs. of rosin, and 200 lbs. of alum to a ton of pulp.

We have discovered that the substantial elimination of lime from the pulp greatly reduces foaming, but some foaming takes place in the paper making machine. This we have also discovered is due to the agitation of the pulp, and the foaming is substantially all eliminated by reducing the agitation to a minimum. This end is attained by making the passage for the flowing pulp wider than usual and of substantially uniform cross section or capacity throughout. In particular, any restriction at the outlet of the passage is avoided.

Straw board, that is board made from straw pulp, is usually made on a machine of the cylinder type, including a suitable tank or vat 1, and a web forming cylinder 2. The pulp flows from the stock pipe 3 into the bottom of the tank at one end thereof, and past a series of baffles 4, 5 and 6 to the cylinder.

Referring to the drawing, it will be seen that the baffles 4 and 6 extend to the bottom of the tank, while the baffle 5 depends from the top. This arrangement provides a tortuous passage from the stock pipe to the cylinder, the pulp flowing as indicated by the arrows.

In the usual practice, the baffle 6 is spaced about two inches from the periphery of the cylinder, and all of the baffles are relatively close, so that a considerable degree of agitation is imparted to the pulp during the flow from the stock pipe to the cylinder. In the present method the agitation is greatly lessened and substantially eliminated, by spacing the baffle 6 at least double the usual distance from the cylinder. That is, the distance is increased to at least four inches, and in addition the baffles 4, 5 and 6 are spaced further apart from each other than usual, and from the end of the tank, for a like reason.

The baffles 4, 5 and 6 are spaced apart equally from each other and from the end of the tank, and the opening between each baffle and the tank wall is of the same cross section as the space between adjacent baffles. The excess of waste water is drawn out through a suction pipe 7 on the inner side of the baffle 6.

This arrangement provides a passage for the pulp of substantially uniform capacity from the stock pipe to the cylinder, and without any restriction at the outlet, so that the flow of the pulp is uniform and with a minimum of agitation at the entrance to the body of the tank, that is between the baffle 6 and the cylinder.

So far as we are aware, we are the first to produce a moisture resistant article of the character in question from straw pulp steam digested in the presence of an alkali.

and particularly wherein the moisture resistant material or size is intimately incorporated with the thoroughly washed pulp fibres during the beating, so that every part of the article is permeated by the size. We are able to produce this article, by the care exercised in the cooking of the pulp, in the elimination of the alkali, and in the substantial elimination of agitation in the flow of the pulp to the web forming cylinder, so that the pulp is devoid of sliminess, and will be picked up by the cylinder. The rosin referred to as in the proportion of 90 lbs. to the ton of stock is the usual prepared rosin size, but the proportion of rosin and the addition of a mordant, such as alum, in about the proportion stated, is we believe, new with us as applied in the manufacture of pulp prepared in the manner and for the purposes herein described.

What is claimed as new is:

1. As a new product of manufacture, water and moisture repellent pulp board formed from straw fibres substantially free from alkali and having a rosin size incorporated therein.

2. As a new product of manufacture, water and moisture repellent pulp board formed from steam digested straw fibres substantially free from alkali and having rosin size and a mordant incorporated therein.

3. As a new product of manufacture, water and moisture repellent pulp board formed from steam digested straw fibres substantially free from alkali and having rosin size and a mordant incorporated therein in about the proportions of 90 lbs. of rosin and 200 lbs. of alum to approximately a ton of pulp.

4. The herein described process of making water and moisture repellent strawboard which consists in steam digesting straw in the presence of an alkali, then thoroughly beating the digested straw to form a pulp, then washing the pulp to remove all or substantially all traces of alkali, then thoroughly incorporating rosin size with the alkali cleansed pulp, and then feeding the pulp quietly and without undue agitation to a pulp-making machine and forming the same into a sheet.

5. The herein described process of making water and moisture repellent strawboard which consists in steam digesting straw in the presence of an alkali, then thoroughly beating the digested straw to form a pulp, then washing the pulp to remove substantially all traces of alkali, then thoroughly incorporating rosin size with the alkali cleansed pulp, then adding a mordant, and then feeding the pulp quietly and without undue agitation to a paper-making machine and forming the same into a sheet.

6. The herein described process of making water and moisture repellent strawboard which consists in steam digesting straw in the presence of an alkali, then thoroughly

beating the digested straw to form a pulp, then thoroughly washing the pulp to remove substantially all traces of alkali, then thoroughly incorporating rosin size and alum with the lime-cleansed pulp in the proportions of about 90 lbs. of rosin and 200 lbs. of alum to approximately a ton of pulp, and then feeding the pulp quietly and without un-

due agitation to a paper-making machine and forming the same into a sheet.

Signed at Terre Haute in the county of Vigo and State of Indiana this 25th day of October, A. D. 1926.

10

EDWARD B. WESTON.  
WILLIAM G. CLARK.